

## UNITED STATES PATENT OFFICE

2,418,629

## AROMATIC HYDROCARBONS AND THEIR HALOGEN DERIVATIVES AS ANTIFOG-GANTS

George E. Fallesen, Rochester, N. Y., assignor to Eastman Kodak Company, Rochester, N. Y., a corporation of New Jersey

No Drawing. Application January 13, 1944,  
Serial No. 518,120

19 Claims. (Cl. 95—7)

1

This invention relates to fog inhibitors for photographic emulsions and to photographic emulsions containing them.

It is known that photographic emulsions, particularly ultra-sensitive emulsions, exhibit a tendency to form a deposit of silver in the unexposed emulsion. This deposit extends more or less uniformly over the entire emulsion and is known as fog. Photographic fog is of two types, local and general. Local fog is formed by exposure of the film or plate at undesired points, as by a light leak in the camera, or by local action of chemicals. General fog or, as it is sometimes known, chemical fog, is formed in a number of ways. It may be caused by the conditions under which the film or plate is stored, such as conditions of high temperature or unusually long time of storage. The nature of the emulsion may also produce chemical fog, as well as conditions of development of the emulsion, as by development for protracted periods of time or at temperatures above normal. Highly sensitive emulsions are more likely to fog than those of lower sensitivity. I am concerned primarily with general or chemical fog.

It is an object of the present invention to provide antifogging or fog inhibiting agents for ultra-sensitive photographic emulsions and thereby to preserve the emulsions against deterioration resulting in fog. A further object is to provide antifogging agents which do not markedly lower the sensitivity of the emulsion. Other objects will appear from the following description of my invention.

These objects are accomplished by developing an exposed silver halide emulsion in the presence of an aromatic hydrocarbon or a halogenated aromatic hydrocarbon. I prefer to use aromatic hydrocarbons of the benzene series having a phenyl substituent or a halogen substituent or a lower alkyl substituent such as a methyl or ethyl substituent.

These compounds may be incorporated in an emulsion to which may be added optical sensitizing dyes. The emulsion may be one which is intended to be used directly after emulsification or one which is subjected to ripening. In some cases the fog inhibiting effect of the hydrocarbons or halogenated hydrocarbons is evident only in unsensitized emulsions or in emulsions which have been stored or incubated for an appreciable period of time.

Hydrocarbons and halogenated hydrocarbons which I have found suitable for use according to my invention, comprise the following examples:





The antifoggant properties of the compounds used according to my invention were tested as follows:

Silver iodobromide was precipitated in 0.8% gelatin solution. After precipitation was complete, this entire volume of emulsion was cooled and divided into portions weighing 1643 grams each. To each portion was added enough gelatin to increase the gelatin concentration to approximately 6.6%. Each portion was then heated to the required digestion temperature, that is, about 60° C. and as soon as this temperature was reached a certain amount of the compound to be tested, e. g., 25 grams of cumene, dissolved in 300 cc. of methyl alcohol, was added. Digestion was then continued for 30 minutes at the specified temperature and the emulsion was then chilled

nating from the same precipitation of silver halide.

After washing, each emulsion was heated to the optimum point for maximum speed and gamma with acceptable fog. Unsensitized and panchromatized samples of each emulsion so finished were coated by machine on glass plates. After the plates were dry, a series of sensitometric tests were made on them. The data were then compared with those of the check emulsion containing no addendum. These tests include initial tests for speed, gamma and fog, made on the day after coating, similar tests on a second set of plates incubated at 120° F., dry heat, for 6 days and a third set of tests made on a third set of plates after having been kept under tropical conditions for 14 days. (The "tropical conditions" are simulated by varying the temperature and humidity through a cycle to reproduce day and night conditions in tropical climates.) Plates for each of these tests were developed for 3 minutes at 65° F. in Kodak D-19 developer which had the following composition:

|    |                                  |       |     |
|----|----------------------------------|-------|-----|
| 25 | Monomethyl-p-aminophenol sulfate | grams | 2.2 |
|    | Sodium sulfite (desiccated)      | do    | 96  |
|    | Hydroquinone                     | do    | 8.8 |
|    | Sodium carbonate (desiccated)    | do    | 48  |
| 30 | Potassium bromide                | do    | 5   |
|    | Water to                         | liter | 1   |

The results of these tests are tabulated below, in each case the amount of hydrocarbon or halogenated hydrocarbon being 12.5 grams per 1000 cc. of unsensitized wet emulsion.

#### Hydrocarbons

| Name of Compound   | Initial Fog Tests      |                           | Tropical Condition 14-Day Incubation Fog Tests |                           | 6-Day 120° F. Dry Incubation Fog Tests |                           |
|--------------------|------------------------|---------------------------|------------------------------------------------|---------------------------|----------------------------------------|---------------------------|
|                    | Emulsion with Compound | Emulsion without Compound | Emulsion with Compound                         | Emulsion without Compound | Emulsion with Compound                 | Emulsion without Compound |
| Cumene             | .04                    | .05                       | .05                                            | .10                       | .05                                    | .10                       |
| Diethyl benzene    | .04                    | .05                       | .05                                            | .24                       | .05                                    | .10                       |
| Mesitylene         | .03                    | .05                       |                                                |                           | .09                                    | .10                       |
| Pentamethylbenzene | .04                    | .05                       | .05                                            | .24                       | .05                                    | .10                       |
| Pseudocumene       | .04                    | .04                       |                                                |                           | .04                                    | .09                       |
| Toluene            | .04                    | .04                       | .06                                            | .24                       | .06                                    | .10                       |
| Triethylbenzene    | .05                    | .05                       | .05                                            | .24                       | .05                                    | .10                       |
| <i>o</i> -Xylene   | .04                    | .05                       | .05                                            | .24                       | .05                                    | .10                       |
| <i>p</i> -Xylene   | .04                    | .05                       | .05                                            | .24                       | .05                                    | .10                       |

#### Halogenated hydrocarbons

| Name of Compound              | Initial Fog Tests      |                           | Tropical Condition 14-Day 120° F. Incubation Fog Tests |                           | 6-Day 120° F. Dry Incubation Fog Tests |                           |
|-------------------------------|------------------------|---------------------------|--------------------------------------------------------|---------------------------|----------------------------------------|---------------------------|
|                               | Emulsion with Compound | Emulsion without Compound | Emulsion with Compound                                 | Emulsion without Compound | Emulsion with Compound                 | Emulsion without Compound |
| Bromobenzene                  | .07                    | .05                       | .09                                                    | .12                       | .09                                    | .17                       |
| 2-Bromocymene                 | .04                    | .05                       | .05                                                    | .17                       | .04                                    | .12                       |
| Bromomesitylene               | .03                    | .05                       | .04                                                    | .17                       | .05                                    | .12                       |
| Bromostyrene                  | .03                    | .05                       | .06                                                    | .17                       | .05                                    | .12                       |
| <i>o</i> -Bromotoluene        | .09                    | .09                       | .09                                                    | .14                       | .16                                    | .24                       |
| 1,2,4,5-Tetrabromobenzene     | .07                    | .09                       | .06                                                    | .14                       | .08                                    | .24                       |
| <i>p</i> -Phenylethylbromide  | .04                    | .05                       | .04                                                    | .17                       | .04                                    | .12                       |
| Iodobenzene                   | .05                    | .05                       | .20                                                    | 1.2+                      |                                        |                           |
| Fluorobenzene                 | .05                    | .06                       |                                                        |                           | .09                                    | .13                       |
| <i>o</i> -Fluorochlorobenzene | .04                    | .05                       | .05                                                    | .14                       |                                        |                           |

<sup>1</sup> 8 weeks under tropical conditions.

and stored in preparation for shredding and washing. One of these portions received no additions other than the required gelatin and it served as the control for all the portions origi-

75 The amount of fog was determined by reading the density on the unexposed area of the test after exposure and development of the emulsion in the usual manner.

In the method of testing the emulsions described above, the hydrocarbons or halogenated hydrocarbons were introduced into the emulsion immediately after precipitation of the silver halide and after the emulsion had been raised to the digestion temperature but before digestion was complete. I have also found that bromohydrocarbons may be added to the emulsions after washing and before finishing and that, when added at this stage, they stabilize the sensitivity of panchromatic emulsions. This stabilization of panchromatic sensitivity is in addition to the antifoggant properties which the compounds possess. Ordinarily the emulsion, after digestion, is chilled, shredded and washed and, when ready for coating, is heated to the optimum point for maximum speed and gamma with acceptable fog. The emulsion is then coated or dried. If the bromohydrocarbon is added to the emulsion just prior to this heating to which the emulsion is subjected before coating, the panchromatic sensitivity of the emulsion is retained for a greater period of time upon storage of the emulsion. The effect of the bromohydrocarbons in stabilizing the red sensitivity of an emulsion was tested by preparing a panchromatic emulsion in the usual way as described above but without addition of an antifoggant. Bromomesitylene was then added in varying amounts to portions of the emulsion just prior to finishing, that is, prior to the heating step to which the emulsion was subjected before coating and plates were coated from these various portions of the emulsion. The plates were then kept for 8 weeks under tropical conditions and were then exposed on a sensitometer and developed in Kodak D-19 developer. The check emulsion to which no bromohydrocarbon had been added lost 45% of its speed whereas the loss in emulsions to which bromomesitylene had been added ranged from 12 to 22%. The fog was also lower in the emulsions to which the bromomesitylene had been added than in the check emulsion.

The following table shows the results obtained upon adding bromomesitylene to the emulsion in this way, the percentage of original speed of the emulsions and the fog in the various coatings being recorded in the table.

| Amount                 | Percent of Original Speed | Fog |
|------------------------|---------------------------|-----|
| 1.5 g. per liter.....  | 80                        | .14 |
| 3 g. per liter.....    | 78                        | .14 |
| 6.3 g. per liter.....  | 83                        | .12 |
| 12.5 g. per liter..... | 88                        | .11 |
| Check.....             | 55                        | .19 |

The fog inhibiting agents which I have described may be used in various kinds of photographic emulsions. In addition to being useful in ordinary non-sensitized emulsions, some of them may be used in orthochromatic, panchromatic and X-ray emulsions. Various silver salts may be used as the sensitive salt such as silver bromide, silver chloride, silver bromoiodide, and silver chlorobromide. The dispersing agent may be gelatin or other suitable colloid, such as collodion, albumen, cellulose organic derivatives or synthetic resins.

It is known that synthetic waxes, such as chlorinated naphthalenes and chlorinated diphenyls have been used as lubricants in photographic emulsions. I do not use such materials, but employ halogenated hydrocarbons which are non-waxy, monomeric compounds of relatively low

molecular weight. The chlorinated hydrocarbon waxes which have previously been used to lubricate film are believed to be polymeric substances.

In addition to their use in the sensitive emulsion itself, my fog inhibiting agents may also be incorporated in an overcoating or intermediate layer in the photographic element containing the sensitive emulsion layer.

It is to be understood that I contemplate as included within my invention all modifications and equivalents falling within the scope of the appended claims.

I claim:

1. A gelatino-silver halide emulsion containing a fog-inhibiting amount of a non-waxy aromatic hydrocarbon of the benzene series having a substituent selected from the class consisting of halogen atoms, an unsubstituted phenyl radical, unsubstituted lower alkyl radicals, and halogen substituted lower alkyl radicals, said hydrocarbon being free from other substituent groups.

2. A gelatino-silver halide emulsion containing from 1-15 grams per liter of wet emulsion of a non-waxy aromatic hydrocarbon of the benzene series having a substituent selected from the class consisting of halogen atoms, an unsubstituted phenyl radical, unsubstituted lower alkyl radicals and halogen-substituted lower alkyl radicals, said hydrocarbon being free from other substituent groups.

3. The method of reducing the amount of fog produced upon development of a silver halide emulsion which comprises developing said emulsion in the presence of a fog-inhibiting amount of a non-waxy aromatic hydrocarbon of the benzene series having a substituent selected from the class consisting of halogen atoms, an unsubstituted phenyl radical, unsubstituted lower alkyl radicals, and halogen-substituted lower alkyl radicals, said hydrocarbon being free from other substituent groups.

4. A gelatino-silver halide emulsion containing a fog-inhibiting amount of a non-waxy halogen-substituted aromatic hydrocarbon of the benzene series free from other substituent groups.

5. A gelatino-silver halide emulsion containing a fog-inhibiting amount of a bromobenzene.

6. A gelatino-silver halide emulsion containing a fog-inhibiting amount of a fluorobenzene.

7. A gelatino-silver halide emulsion containing a fog-inhibiting amount of a non-waxy aromatic hydrocarbon of the benzene series having an alkyl substituent group selected from the class consisting of methyl and ethyl groups, and free from other substituent groups.

8. A gelatino-silver halide emulsion containing a fog-inhibiting amount of a methylbenzene.

9. A gelatino-silver halide emulsion containing from 1 to 15 grams per liter of wet emulsion of a non-waxy halogen-substituted aromatic hydrocarbon of the benzene series free from other substituent groups.

10. A gelatino-silver halide emulsion containing from 1 to 15 grams per liter of wet emulsion of a bromobenzene.

11. A gelatino-silver halide emulsion containing from 1 to 15 grams per liter of wet emulsion of a fluorobenzene.

12. A gelatino-silver halide emulsion containing from 1 to 15 grams per liter of wet emulsion of a non-waxy aromatic hydrocarbon of the benzene series having an alkyl substituent group selected from the class consisting of methyl and

methyl groups, and free from other substituent groups.

13. A gelatino-silver halide emulsion containing from 1 to 15 grams per liter of wet emulsion of a methylbenzene.

14. The method of reducing the amount of fog produced upon development of a silver halide emulsion, which comprises developing said emulsion in the presence of a fog-inhibiting amount of a non-waxy halogen-substituted aromatic hydrocarbon of the benzene series free from other substituent groups.

15. The method of reducing the amount of fog produced upon development of a silver halide emulsion, which comprises developing said emulsion in the presence of a fog-inhibiting amount of a bromobenzene.

16. The method of reducing the amount of fog produced upon development of a silver halide emulsion, which comprises developing said emulsion in the presence of a fog-inhibiting amount of a fluorobenzene.

17. The method of reducing the amount of fog produced upon development of a silver halide emulsion, which comprises developing said emulsion in the presence of a fog-inhibiting amount of a non-waxy aromatic hydrocarbon of the benzene series having an alkyl substituent group selected from the class consisting of methyl and ethyl groups, and free from other substituent groups.

18. The method of reducing the amount of fog produced upon development of a silver halide emulsion, which comprises developing said emulsion in the presence of a fog-inhibiting amount of a methylbenzene.

19. The method of inhibiting fog in, and stabilizing the sensitivity of, an optically-sensitized gelatino-silver halide emulsion, which comprises precipitating the silver halide in the gelatin, 10 optically sensitizing said emulsion, digesting the emulsion at an elevated temperature, chilling and washing said emulsion, mixing with said emulsion a fog-inhibiting amount of bromomesitylene, and heating said emulsion to a temperature producing maximum speed and contrast with minimum fog.

GEORGE E. FALLESEN.

#### REFERENCES CITED

20. The following references are of record in the file of this patent:

#### UNITED STATES PATENTS

| Number       | Name                  | Date          |
|--------------|-----------------------|---------------|
| 25 1,763,990 | Sheppard et al. _____ | June 17, 1930 |
| 2,046,067    | Gaspar _____          | June 30, 1936 |
| 2,150,702    | Sheppard et al. _____ | Mar. 14, 1939 |
| 2,158,204    | Sheppard et al. _____ | May 16, 1939  |
| 2,238,632    | Dersch et al. _____   | Apr. 15, 1941 |
| 2,288,586    | Dersch et al. _____   | June 30, 1942 |
| 2,333,766    | Crabtree et al. _____ | Nov. 9, 1943  |